

April 7, 1931.

E. BURKE

1,799,580

INSULATOR

Filed Feb. 7, 1927



## UNITED STATES PATENT OFFICE

EDMUND BURKE, OF PORTLAND, MAINE, ASSIGNOR TO BROWN COMPANY, OF PORTLAND, MAINE, A CORPORATION OF MAINE

## INSULATOR

Application filed February 7, 1927. Serial No. 166,538.

My present invention relates to insulators and is of particular importance in connection with insulators for high tension installation. Such insulators as are at present used for this work are enormously expensive and are of such a fragile nature that they are frequently broken in shipping and handling or are peculiarly objects of vandalism as by sniping. This all contributes to a very heavy installation and upkeep cost and to great trouble and annoyance in maintaining efficiency on the lines.

It has been proposed to make composition insulators of less expensive material and some of the smaller and simpler types of insulators have been so produced. The problem, however, of producing a suitable insulator for high tension lines and one capable of being produced with sufficient resistance and tensile strength has not as far as I know been solved. The problem includes that of producing insulator structures of a tensile strength sufficient to withstand many thousand pounds and at the same time being able to withstand the sparking and arcing effects of the highest voltages.

Considering first the material phase of my invention I secure a tensile variant while preserving dielectric strength. As hereinbefore pointed out I effect this by the use of a substantially homogeneous material in two forms each old in itself and both heretofore used together but I use them in a new relation and according to a new concept of their potentialities.

Briefly, this aspect of my invention relates to the use of a fibrous material in two forms—both permeable by a dielectric binder but differentiated as to permeability and tensile strength. The combining possibilities give in this art that factor much needed and long sought by which commercial success may be attained.

In dealing with my other factor (structural) I provide a stem member of general

construction and capable of being manufactured from such a fibre mixture in commercial lengths.

By combining with this unitary elements, say of the petticoat type, I am able to produce insulators varying from the single unit type to those of maximum total distances capable of insulating against the highest voltages.

For convenience of illustrative reference, I have selected certain well known types of insulators and have shown in the accompanying drawings embodiments in accordance with my invention in such insulators. In the drawings:

Fig. 1 is a general elevation of a multiple suspension type of insulator.

Fig. 2 is a fragmentary section thereof.

Fig. 3 is a sectional view of a pin type insulator, and

Fig. 4 is a sectional detail of a terminal connection.

Referring to Fig. 1, I have indicated at 1 a tubular stem formed preferably of a fibrous mixture. In the form shown, this is turned with an exterior thread and the petticoat units 2 are threaded thereon preferably being pinned as at P by wooden pegs as indicated in Fig. 2.

Such an insulator as shown in Fig. 1 may have the usual upper eye connection 3 screwed on to the end of the tube and a lower clevis connection screwed on the other end as indicated at 4. The tubular member 1 is preferably filled with a high melting point pitch, as indicated at 5. Any desirable pitch or asphaltic material may be used for this purpose, as for example gilsonite.

Where the central stem is to be used in the general pin type of insulator I provide as in Fig. 3, a stem 1<sup>1</sup> threaded as before but turned so as to give a butt 1<sup>2</sup> in which is formed a threaded socket 6 corresponding to the usual construction of such insulators. Such an insulator, I have illustrated in Fig. 3, has its terminal 7 provided with cable notches and

grooves 7<sup>1</sup> and 7<sup>2</sup>, respectively. In the form shown in Fig. 3, the petticoat units 2<sup>1</sup> are provided with short necks 2<sup>2</sup> by which the units are spaced from each other.

- 5 In Fig. 4 I have shown a convenient structure in the manufacture of stems for insulator purposes. In this drawing I have indicated the tubular stem by 1. This may be a piece of fibre tubing which can be produced in 10 stock lengths and sizes. On the end of such a section 1 I slip a short section 10 cut from a tubing having an internal diameter substantially fitting the external diameter of the tube 1. This ring 10 is preferably pinned as 15 at P by wooden pins thus forming on the tube 1 a shoulder for carrying any suitable terminal member as 9 having engaging arms or points 8. The pins P are preferably of wood as such pins are capable of receiving water- 20 proofing and dielectric impregnation.

In such structures it is to be noted that there are two main members, each of which must be of high dielectric strength but when considered as separate elements only one need be of 25 considerable tensile strength.

This apparently has been one of the failures of previous concepts relating to composition insulators. One of the problems involved was that of providing substantial homogeneity throughout the mass of the material from which the insulator is formed. This is important as a matter of securing high dielectric strength and is also important as a matter of ultimate bonding or consolidation of the separate members so as to secure 30 a substantial unification. Having therefore understood the possibilities of a specially developed stem member, my concept was of a stem of substantially the same material as the 35 flange or petticoat portions but of a much higher tensile strength and one capable of being turned or threaded or otherwise worked on to get such mechanical assembly as seemed desirable.

40 I therefore preferably take two classes of the same material, as for example long wood fibre and fine sawdust or wood flour. I find it preferable to have these of generally the same origin, although it is possible to substitute fibre of proper length of other origin than a woody origin, as for example leather fibre or even such vegetable fibres as cotton. While the wood pulp is preferable for many 45 reasons, there might be adulteration or substitution by the use of infusorial earths, cork, finely ground clinkers or a great variety of other materials. I mention these in order that there may be no misunderstanding as to the scope of my invention, but on account 50 of the inexpensive character of woody matters and their general availability, such seem to me at present to be logical materials for commercial production.

55 In preparing such materials I utilize the two forms generally as follows. For my

stem mixture I use preferably a long strong fibre such as the best quality of spruce and preferably a selected fibre. Such fibre takes a high impregnation and when mixed with wood flour, which is even more easily impregnated, I am able to get a stem mixture of very great strength. The amount of the long fibre used merely depends on the ultimate strength of the stem required and the mixture may be infinitely varied from a low 70 percentage of long fibre to an exclusive use of long fibre which makes a material of very great tensile strength. Such a stem is capable of being turned and threaded as indicated in the drawings and when produced in tubular 75 form is capable not only of fibre impregnation but of secondary impregnations externally and internally and may then be filled with a fused or melted core of the same dielectric or any variant desired. In making 80 the flange or petticoat members where the tensile strength is not needed, the fibre may be omitted and the wood flour or like material impregnated or moulded rapidly and shaped.

The insulator is then assembled in its 85 several parts and preferably dipped in a moulten bath of high melting point pitch or mixture. Such a coating not only completes the assembly and unifies the parts, but by reason of its impregnation of all cracks or 90 exposed surfaces resulting from manufacture gives the resultant article a high finish, weather resistant surface, and makes of the 95 assembly a unit of very high electrical resistance.

100 The stem principle as applied to such structures makes possible a very extended total distance of insulation and makes possible a very rapid assembly of elementary parts into a variety of insulators each when 105 completed constituting substantially a dielectric entirety.

The filling as indicated at 5 not only makes 110 possible the use of the tubular stem with all its manufacturing advantages, but actually makes out of that stem a member of greater insulating value which in itself would be important apart from the strength and economy gained by the use of the tubular principle for the stem.

115 While applicant has only attempted to show two general types of insulators, it will be understood that most of the usual types and designs of insulators can be made in accordance with my invention and that such variations in design and other variations in 120 details of structure and assembly are all understood to be within the purview of his invention as defined in the appended claims.

125 What I therefore claim and desire to secure by Letters Patent is:—

1. In an impregnated insulator, a stem member composed of long wood fibre and a comminuted absorbent filler, and a flange member having a greater amount of said ab- 130

sorbent filler and a lesser amount of long fibre, and a non-conductive core sealed within said stem.

2. In an impregnated insulator, a stem member composed of long wood fibre and a comminuted absorbent filler, and a flange member having a greater amount of absorbent filler and a lesser amount of said long fibre.

10 In testimony whereof I affix my signature.  
EDMUND BURKE.

15

20

25

30

35

40

45

50

55

60

65